

## UNITED STATES PATENT OFFICE

2,063,857

## LUBRICATING OIL

Waldo L. Steiner, Ponca City, Okla., assignor, by  
mesne assignments, to The Lubri-Zol Develop-  
ment Corporation, Cleveland, Ohio, a corpora-  
tion of Delaware

No Drawing. Application February 10, 1934,  
Serial No. 710,732

## 5 Claims.

(Cl. 87—9)

My invention relates to lubricating oils and more particularly to improved methods for the production of high quality lubricating oils and such products as new compositions of matter.

5 The present trend of development in the automotive industry toward speedier and more powerful motors has made the development of higher film strength lubricants a necessity. Some manufacturers are partially getting around this necessity, momentarily at least, by increasing the area 10 of bearing surfaces and plating cylinder walls with such metals as tin, chromium, copper and the like. These plating methods have not proved entirely satisfactory and the products obtained 15 by these plating methods do not stand up as desired in commercial use. Manufacturers fully realize that the lubricants that are now found on the market are not entirely satisfactory for the present day motors and will be still less so for 20 the motors of the future. The very best quality hydrocarbon lubricants do not have sufficient film strength to stand up under the severe load imposed by motor designs. When the film of lubricants between the rubbing surfaces breaks down 25 due to its lack of extreme pressure characteristics, there is metal-to-metal contact at the rubbing surfaces, with subsequent scratching, scuffing, and seizure of the metals.

The most important property of a lubricant 30 which is to perform under thin film conditions is its film strength, which may be defined as the maximum weight or load which can be applied to rubbing surfaces lubricated by the lubricant before actual metal-to-metal contact occurs with 35 subsequent seizure of the parts. The film strength of a lubricant may be determined by a test machine which operates under a given set of conditions, such as rubbing speed, oil temperature, etc. but under varying loads. The Timken machine 40 developed and described by the Timken Roller Bearing Company is probably the best test machine of this type now in use, because it gives reproducible results.

45 One object of my invention is to provide a lubricating oil of high film strength.

My invention may be described in outline, as a 50 method of producing high film strength lubricating oils by the addition of small amounts of a halogenated terpene, such as, pinene hydrochloride to hydrocarbon lubricants and the product resulting from such addition as a new composition of matter.

The following example of my invention will act as an illustration of one embodiment of the in-

vention, but it is to be understood that my invention is not limited to the examples given.

One per cent of pinene hydrochloride by volume, prepared by the ordinary laboratory method of saturating pinene with dry hydrochloric acid, 5 added to an S. A. E. 30 mineral lubricating oil by thoroughly mixing together at a temperature of about 160° F. will, when tested on the Timken machine, give a film strength of approximately 11,500 pounds per square inch at the rubbing surface. Another sample of the same mineral oil before being blended with the pinene hydrochloride will give a film strength of approximately 10 6,000 pounds per square inch at the rubbing surface. The improvement, it will be noted, is approximately 15 100%.

Smaller or larger percentages of pinene hydrochloride may be used varying from .1% to 10.0% with varying effects on the film strength. Those skilled in the art can determine the percentage of 20 pinene hydrochloride to be added when the knowledge of the film strength of the original hydrocarbon lubricant is available and knowing the desired film strength of the finished product.

This invention does not cover any specific 25 means of halogenating pinene and the like, since any of the well-known methods of halogenation may be employed. The percentage of halogen to be added to the pinene may be varied over rather wide limits, depending upon the desired results 30 after blending with mineral lubricants. As little as 5% of halogen by weight in the pinene may be used in some instances and quantities as great as 50% by weight of halogen in the pinene or more 35 may be used in other instances.

Halogen derivatives of other terpenes may be 40 employed in the ambit of my invention, but halogenated pinene is one preferred terpene, because of its relative cheapness and stability when added to hydrocarbon lubricants.

45 Halogens other than chlorine, which was used in the example, may be used. Fluorene is somewhat difficult to handle and bromine and iodine are very expensive. As chlorine is much cheaper and readily available on the market, it is the preferred halogen to be used in my invention.

Halogenated terpenes may be added to any type 50 of lubricant and my invention is not restricted to lubricants of any classification and includes hydrogenated and synthetic lubricants. My invention is not limited to crank case oils, since any lubricant for any use is greatly improved by increasing its film strength.

It will be understood that certain features, sub-combinations and operations are of utility and 55

- may be employed without reference to other features and sub-combinations. This is contemplated by and is within the scope of my claims. It is further obvious that various changes may be  
5 made in details, within the scope of my claims, without departing from the spirit of my invention. It is therefore, to be understood that my invention is not to be limited to the specific details described.  
10 Having thus described my invention what I claim is:  
1. A lubricating oil comprising in combination a hydrocarbon oil and a small quantity of a halo-  
genated terpene.

2. A lubricating oil comprising in combination a hydrocarbon oil and a small quantity of a chlorinated terpene.  
3. A lubricating oil comprising in combination a hydrocarbon oil and a small quantity of halo- 5 genated pinene.  
4. A lubricating oil comprising in combination a hydrocarbon oil and a small quantity of chlorinated pinene.  
5. A lubricating oil comprising in combination 10 a hydrocarbon oil and a small quantity of pinene hydrochloride.

WALDO L. STEINER.